

## UNITED STATES PATENT OFFICE

2,113,325

PROCESS AND COMPOSITION FOR TREAT-  
ING NATURAL AND ARTIFICIAL FIBERSTheodoor Koch, Oosterbeek, Netherlands, as-  
signor to American Enka Corporation, Enka,  
N. C., a corporation of DelawareNo Drawing. Application March 3, 1936, Serial  
No. 66,967. In Germany March 12, 1935

2 Claims. (Cl. 19—66)

This invention relates to the treatment of natural and artificial fibers composed principally of cellulose or of cellulosic origin. More particularly the present invention contemplates softening and finishing cellulosic fibers to produce an increased and superior suppleness and flexibility in the thread.

In order to properly condition threads of both natural and artificial origin for weaving and knitting purposes, it is necessary to subject the thread to numerous handling operations which necessitate employing a protective medium; and during knitting and weaving stages the friction on the thread must be reduced to a minimum while at the same time a high degree of pliability is desired.

It is known to apply certain oily and fatty compositions to threads for lubrication purposes to thereby decrease the friction between the threads themselves and between the threads and mechanical parts with which they come in contact. However, prior to the present invention, it has been impossible simultaneously to effect the desired amount of suppleness in the thread. The basic reason why the oils and fats formerly employed did not improve the suppleness of the threads to a very high degree is not completely known. However, it appears reasonable to assume that the reason resides in the chemical properties of the oil and the cellulose. Cellulosic compositions are strongly hydrophilic, i. e., capable of absorbing moisture, whereas the oils are hydrophobic, i. e., will not absorb moisture to such a marked extent. For this reason it seems evident that fibers consisting of cellulose only absorb oils or fats to a small extent. When such hydrophilic fibers are treated with the hydrophobic oils then the oils are primarily held in the form of a film on the outside of the fibers and are absorbed into the body of the fibers to a very slight degree only.

It is, therefore, the object of the present invention to provide a process for softening and finishing cellulosic fibers having a high degree of suppleness and pliability.

A further object of the invention is to treat threads and the like with a composition which will reduce the frictional contact on the thread to a minimum.

The invention further contemplates the utilization of an improved and novel composition for imparting to the threads the desired properties.

Other objects and advantages will be apparent by referring to the following detailed description.

It has now been determined that an improved process and product is produced if fibers consisting essentially of cellulose are impregnated with a finishing agent having both hydrophobic and hydrophilic properties. These combined properties render the thread treated therewith both pliable and less frictionable. Finishing agents having the necessary prerequisites have now been found to be the partly saponified esters of polyvalent alcohols and higher fatty acids which still contain free hydroxyl groups. For example, those compositions may be mentioned having more than eight carbon atoms, although in some cases this may not be essential. These esters contain unesterified hydroxyl groups which groups are hydrophilic and accordingly impart an increased suppleness to the thread while the lubricating properties are in no way impaired. The mono- and diglycerides of higher fatty acids have been found to be particularly adaptable to the present invention, as they have in addition to the aforementioned advantages, the property of emulsifying readily in water without the addition of emulsifying agents per se. This property renders the thread or fabric manufactured therefrom susceptible to subsequent simple treatments whereby the composition is easily removed without the usual extensive scouring operations.

Examples of the specific materials which may be employed in this process are glycol monooleate, glycerin distearate, erythrit tripalmitate and the like. Further mixed esters of polyvalent alcohols which contain unesterified hydroxyl groups may be used such as glycerin-1-palmitate-3-oleate.

The fatty acid esters with free unesterified hydroxyl groups may be manufactured by several methods such as by esterifying fatty acid anhydrides with polyvalent alcohols, by double decomposition of chlorhydrins with fatty acid salts, by heating natural triglycerides with polyvalent alcohols or their alkyl ethers with more than one free hydroxyl group (with or without the addition of a catalyst), or by fractionated saponification of glycerides.

In addition to the materials mentioned above, combined fatty acids of the type oxy-fatty acids may be employed such as acetyl ricinoleic fatty acids which contain esterified hydroxyl groups. Other oxy-fatty acids adaptable for use are estolides fatty acids, fatty acids of blown oils, polymerized fatty acids, and fatty acids with several carboxyl groups.

All of the materials mentioned above may be used in emulsion form or dissolved in the proper

5

10

15

20

25

30

35

40

45

50

55

solvents. They can also be used in various combinations with the fats, waxes, mineral oils, soaps, sulphonated products, et cetera.

*Example 1.*—Natural or artificial fibers consisting essentially of cellulose are immersed in an aqueous emulsion which contains 5% glycerine mono-oleate. After complete impregnation the fibers are taken out of the bath and the excess fluid is removed by hydro-extraction and finally 10 dried by any suitable means.

*Example 2.*—A yarn consisting of a mixture of cotton and artificial silk staple fibers is dressed with a solution containing 3% oil dissolved in a mixture of acetone and sufficient water to produce a homogeneous solution. The oil is prepared by heating 100 parts olive oil and 22 parts glycerine in a vacuum to 175° C. until the product 15 has a saponification number of approximately

155. If desired, a catalyst may be employed. The yarn, having been dressed, is centrifuged and dried in the usual manner.

The above examples are given merely to specify improved compositions to be employed in the present process and it is to be understood that they do not limit the spirit and scope of the present invention.

What I claim is:

1. A process for softening and finishing cellulose fibers comprising treating said fibers with a dilute aqueous acetone solution of glycerine mono-palmitate mono-oleate. 10

2. A process for softening and finishing cellulose fibers comprising treating said fibers with a 15 3% aqueous acetone solution of glycerine mono-palmitate mono-oleate.

THEODOOR KOCH.